

No. 625,863.

Patented May 30, 1899.

E. WOHLWILL.

PROCESS OF OBTAINING CHEMICALLY PURE GOLD.

(Application filed June 4, 1896.)

(No Model.)

2 Sheets—Sheet 1.

Fig. 1.



Witnesses  
B. S. Ober  
P. W. Sommers

Inventor,  
Emil Wohlwill  
By *Henry W. Wohlwill*

No. 625,863.

Patented May 30, 1899.

E. WOHLWILL.

## PROCESS OF OBTAINING CHEMICALLY PURE GOLD.

(Application filed June 4, 1896.)

(No Model.)

2 Sheets—Sheet 2.



Fig. 2.

Witnessed  
B. J. Ober  
B. H. Sommers

Inventor  
Emil Wohlwill.  
By Henry W. Allen, atty.

# UNITED STATES PATENT OFFICE.

EMIL WOHLWILL, OF HAMBURG, GERMANY.

## PROCESS OF OBTAINING CHEMICALLY-PURE GOLD.

SPECIFICATION forming part of Letters Patent No. 625,863, dated May 30, 1899.

Application filed June 4, 1896. Serial No. 594,339. (No specimens.)

*To all whom it may concern:*

Be it known that I, EMIL WOHLWILL, a subject of the German Emperor, residing at Hamburg, Germany, have invented an Improved 5 Process of Obtaining Chemically-Pure Gold from Fine Gold and Alloys Rich in Gold; and I do hereby declare the following to be a full, clear, and exact description of the invention.

This invention has relation to the electrolytic extraction of gold from so-called "refined gold" obtained by affinage or otherwise and which still contains other metals in various proportions or from alloys rich in gold.

The invention has for its object a process 10 whereby the whole of the gold contained in the material to be used as anode is obtained in the form of chemically-pure gold and whereby the process of extraction can be commercially carried out and other valuable 20 metals alloyed with the gold readily recovered.

As is well known, in the chemical separation of gold from impure gold or from alloys of gold the gold is dissolved out of the disintegrated impure gold or alloy by means of aqua regia, and from the clear dilute solution the gold is precipitated by means of a suitable precipitant, while in the electrolytic extraction the dissolution of the gold and its extraction 30 from the solution are effected simultaneously, as is the case in the electrolytic extraction of copper and silver. To this end it is necessary during the electrolytic decomposition of the gold solution used as an electrolyte that a quantity of gold equal to that deposited at the cathode be carried into the electrolyte under the influence of the gold ion or compounds thereof separated at the anode, so that in an uninterrupted extraction the 40 amount of gold in the electrolyte will at all times be approximately the same. When, however, the electrolytic extraction of gold is carried out with an electrolyte containing chlorid of gold and under conditions that give 45 rise to the evolution and liberation of gaseous chlorin at the anode, an amount of anode gold or gold compound proportionate to or corresponding with the amount of gaseous chlorin liberated will remain unaffected by 50 the electrolytic action. It is therefore essential in the profitable and economical extraction of gold by electrolysis that the evolu-

tion of gaseous chlorin at the anode should be avoided. It is furthermore obvious that the electrolytic extraction of the precious 55 metal is most economically effected with currents of comparatively high density, as the dissolution of the anode gold or compound and the precipitation of the pure gold at the cathode are thereby materially expedited. If, 60 however, a solution of gold chlorid in presence of an anode of gold or of a compound or alloy thereof is electrolyzed under the action of an electric current, and especially of a current of comparatively high density, it will be 65 found that there is an essential departure in the behavior of the gold from that of copper or silver under like conditions.

While it is practically immaterial in the continuous carrying over of the anode copper 70 or silver to the electrolyte whether the latter is neutral or more or less acid or more or less concentrated or more or less heated, these factors have a decided influence upon the electrochemical dissolution of gold or its compounds or alloys, which is more pronounced 75 when currents of comparatively high density are used. Thus, for instance, if a neutral pure gold-chlorid solution of normal temperature is electrolytically decomposed in the presence of gold electrodes by the action of a current of as low a density as ten amperes per square meter the free chlorin evolved at the anode will escape without action upon the metal, and this condition is not changed by 80 merely increasing the temperature of the electrolyte. This is also the case with currents of higher density, but still much below one hundred amperes per square meter, when a slightly-acid electrolyte is used, such as may, 85 for instance, be obtained by the evaporation of a solution of gold in aqua regia. I have, however, discovered that the disturbing evolution and escape of chlorin at the anode are not only materially reduced, but absolutely 90 avoided, whenever the electrolyte contains sufficient hydrochloric acid. I have found that at a given temperature the maximum current density at which the whole of the chlorin evolved at the anode is bound corresponds 95 with the quantity of the hydrochloric acid present in the electrolyte, or vice versa, and that this maximum of current density and of chlorin to be bound can be increased in pro-

- portion as the hydrochloric acid contained in the electrolyte is increased and that a further and very material increase takes place when the temperature of the electrolyte is increased 5 relatively to a given percentage of hydrochloric acid therein. Hence if at a given temperature of the electrolyte containing a given quantity of hydrochloric acid the current density is increased beyond the corresponding 10 maximum density an amount of free chlorin corresponding with this increase in current density above the maximum will escape at the anode, which can, however, be prevented either by a corresponding increase in the percentage of hydrochloric acid added to the electrolyte or by increasing the temperature of the latter. My experiments have conclusively proven that in this manner it is possible to continuously operate with comparatively 15 weak solutions of gold chlorid and with currents of a density as high as one thousand amperes per square meter and even higher through the combined influence of high temperature and added hydrochloric acid.
- 20 The invention therefore consists, essentially, in the electrolytic purification of impure gold and of gold alloys by employing as an electrolyte solutions of chlorid of gold containing hydrochloric acid in sufficient quantity to bind the chlorin evolved at the anode or gold-chlorid solutions of a sufficiently high temperature and containing sufficient hydrochloric acid to bind the free chlorin evolved at the anode.
- 25 The fact stated above, that the amount of gold or a compound or alloy thereof dissolved at the anode is proportionate to the amount of hydrochloric acid present in the solution and capable of preventing the escape of gaseous chlorin, will readily be understood from the following: The belief has prevailed that in the known processes of dissolving gold the chlorid ( $\text{AuCl}_3$ ) is obtained; but this cannot be proved in any manner. After a thorough 30 examination into the combinations of gold published by Julius Thomsen (*Thermochemische Untersuchungen*, Vol. 3, p. 382, *et seq.*, Leipsic, 1883) there are but two ways of obtaining chlorid of gold, ( $\text{AuCl}_3$ .) First, finely-divided gold is acted upon with gaseous chlorin of from  $200^\circ$  to  $300^\circ$ , whereby  $\text{Au}_2\text{Cl}_4$  is obtained, which in water splits up into  $\text{AuCl}_3$  and  $\text{AuCl}$ . Second, protochlorid of gold ( $\text{AuCl}$ ) is heated for some time in water, when it splits up in accordance with the following equation:
- 3  $\text{AuCl} = 2\text{Au} + \text{AuCl}_3$ .
- The  $\text{AuCl}_3$  obtained in both cases may be recognized by the fact that it forms with water a brownish-red solution, the thicker layers of which appear black. If this solution is mixed with a suitable quantity of hydrochloric acid, it assumes a yellow color, in that in accordance with the following equation
- 65  $\text{AuCl}_3 + \text{HCl} = \text{AuCl}_3\text{HCl}$
- the double chlorid of gold and hydrogen, des-

ignated by Berzelius as the "acid gold chlorid," is formed. This combination is formed under the evolution of considerable heat, (see 70 Thomsen referred to, Vol. 3, p. 392,) which proves that after the formation of  $\text{AuCl}_3\text{HCl}$  hydrochloric acid has disappeared, and this is shown by the fact that chlorin is not separated when a concentrated solution of  $\text{AuCl}_3\text{HCl}$  is 75 reacted upon with nitric acid, (which would occur if free hydrochloric acid were present,) and hence does not dissolve gold. If the solution of  $\text{AuCl}_3\text{HCl}$  is evaporated to dryness, crystals are formed of the composition  $\text{AuCl}_3$  80  $\text{HCl} + 4\text{H}_2\text{O}$ , which give up the  $\text{HCl}$  only at higher temperatures, the  $\text{AuCl}_3$  being split up into  $\text{AuCl}$  and  $2\text{Cl}$ . Besides this the compound  $\text{AuCl}_3\text{HCl}$  has the properties of a mono-basic acid, and it is therefore correct to write 85 it  $\text{HAuCl}_4$ . There can be no doubt that in each direct solution of gold by chemical means this compound  $\text{HAuCl}_4$  is simultaneously formed and passes over into the solution. If, for instance, gold is dissolved in aqua regia, 90 a yellow solution is obtained, from which crystals of the given composition  $\text{AuCl}_3\text{H} + 4\text{H}_2\text{O}$  are obtained. It must therefore be concluded that of each four parts of the reacting hydrochloric acid in the aqua regia three are always 95 used up in the formation of chlorin and there-through the chlorination of the gold, while the fourth part is used up in an undecomposed condition in the formation of  $\text{HAuCl}_4$ , so that the reactions which take place may be briefly 100 expressed by the following equations:

1.  $\text{HNO}_3 + 3\text{HCl} = 3\text{Cl} + 2\text{H}_2\text{O} + \text{NO}$ .
2.  $\text{Au} + 3\text{Cl} + \text{HCl} = \text{HAuCl}_4$ .

It may be assumed—and this is the general 105 opinion—that the process expressed in Equation 2 comprises two successive reactions, and that the action of the chlorin evolved from the aqua regia upon the gold will form a neutral gold chlorid in accordance with the following equation:



and that through the excess of undecomposed hydrochloric acid, owing to the great affinity 115 of both substances, the double chlorid of gold and hydrogen is formed in accordance with the equation:



It may, however, be assumed that the formation of the compound  $\text{HAuCl}_4$ , according to Equation 2, is only a single indivisible reaction, so that the neutral chlorid of gold does at no time exist or could be supposed to exist as an intermediate step. Both views do clearly show the reactions that take place in the dissolution of gold in aqua regia; but the second only explains also the reactions above referred to and taking place in the electrolytical decomposition of gold-chlorid solutions in the presence of gold electrodes.

If  $\text{AuCl}_3$  were produced by the contact of chlorin with gold, this combination would re-

sult in the absence of hydrochloric acid or another chlorin compound when the chlorin is evolved at the anode under the influence of the electric current and a brownish-red liquid would flow along the anode. That this is not the case, but, on the contrary, that chlorin gas escapes at the anode in the absence of hydrochloric acid or other chlorin compound in the solution, contradicts the assumption that chlorin and gold alone in an aqueous solution can combine and form  $\text{AuCl}_3$ , and yet the conditions during the evolution of chlorin at the anode are the most favorable that could possibly be imagined to the formation of this compound. On the contrary, in accordance with the equation



it follows necessarily that gaseous chlorin escapes without acting on the gold anode when there is a deficiency of hydrochloric acid and that by adding a sufficient quantity of hydrochloric acid the dissolution of the gold anode takes place. The above indivisible equation shows at the same time and quantitatively the factors which are important in the electrolytic dissolution of gold.

The volume of chlorin evolved per second at the anode is determined by the intensity 30 of the current, and this volume is wholly absorbed—that is to say, utilized in the dissolution of gold when there is present at the anode a sufficiency of hydrochloric acid or another chlorin compound, so that the amount 35 of chlorin therein will be equal to at least one-third of that evolved at the anode, this following directly from the equation:



If a less quantity of undecomposed hydrochloric acid is present, a corresponding proportion of chlorin must necessarily escape at the anode.



If undecomposed hydrochloric acid in sufficient quantity is present, so that the proportion of chlorin therein is greater than one-third of the chlorin evolved at the anode, it is possible with a current of higher density—that 50 is to say, under a more copious evolution of chlorin at the anode per second—to bind the whole of the evolved chlorin—i.e., utilize the same for the dissolution of gold.



In a similar manner it follows quite naturally that under an increase of current density, hence under an increase in the volume of chlorin evolved within a unit of time upon a unit of anode-surface, a corresponding increase in the volume of hydrochloric acid will be necessary in order that no chlorin may escape and that the uninterrupted dissolution 65 of the anode may take place.



If the electrolyte composed of  $\text{AuCl}_4\text{H}$  contains no free hydrochloric acid, then, according to Hittorf, (*Poggendorff's Annalen der Physik und Chemie*, Vol. 106, p. 522, *et seq.*), the reactions proceed in such manner that the group  $\text{AuCl}_4$  will be separated at the anode and hydrogen at the cathode and gold only by the secondary effect of such separating 75 hydrogen.



The group  $\text{AuCl}_4$  separated at the anode can- 80 not subsist, and consequently breaks up according to the equation:



Hence chlorin is separated at the anode, in 85 that a reaction in accordance with



cannot take place in an aqueous solution the greater part of the chlorin escapes, and this 90 I prevent, as stated, by the addition of another chlorin compound to the solution, because by this addition the conditions required for the dissolution of gold according to



95

are fulfilled.

The very slight loss in weight of each gold anode, even in solutions apparently free from hydrochloric acid, is perfectly in accord with 100 the above elucidations, because, irrespective of the fact that in accordance with the above Equation 2 hydrochloric acid is formed at the anode and diffuses slowly to the cathode, such acid, besides gaseous chlorin, must be formed 105 in an aqueous solution in which chlorin gas is separated for a certain period of time, always according to the equation:



110

and as a result gold will be dissolved. It is even for this reason that the aqueous solution of chlorin acts as a solvent of gold. The solution does therefore take place in both instances, not because chlorin is capable of dissolving gold without hydrochloric acid, but because it is barely possible to obtain a solution of chlorin free from hydrochloric acid. It is therefore obvious that an addition of hydrochloric acid will prevent the evolution of 115 gaseous chlorin at the anode in the same manner and for the same reasons that a non-decomposed portion of the hydrochloric acid in the dissolution of gold in aqua regia serves to effect the combination of the gold with the 120 chlorin.

In practically carrying out my invention I employ, by preference, as electrolyte a solution containing from about twenty-five to thirty grams of gold per liter and maintain 130 the same during the electrolytic operation at a temperature of from about  $60^\circ$  to  $70^\circ$  centigrade, which electrolyte may contain per liter from about twenty to fifty cubic centimeters,

according to the density of the current used, of fuming hydrochloric acid of a specific gravity of 1.19. In view of the fact that the proportion of hydrochloric acid may become variable during the electrolytic operation by reason of evaporation and consumption any deficiency in acid will manifest itself at once irrespective of any test as to acidity of the electrolyte by the escape of chlorin gas at the anode, and this is to be immediately remedied by the addition of hydrochloric acid until such escape ceases, provided there has been no material reduction in the temperature of the electrolyte. When the temperature of the electrolyte and the quantity of hydrochloric acid therein are in proper accord with the density of the electric current, the bulk of the foreign constituents of the anode will pass into the electrolyte under the influence of the electric current with the anode gold and with these the whole of the platinum and palladium. The major portion of the iridium and other metals of the platinum group remain undissolved, and with these the silver is separated as solid in the form of a chlorid. Similarly a portion of the lead is separated in the form of lead chlorid as soon as the electrolyte becomes saturated therewith, or nearly so, while the bismuth is separated in the form of an oxychlorid should the amount of hydrochloric acid present be insufficient to keep it dissolved. With this insoluble mud, separated at the anode as described and which readily drops off the same in small quantities at a time, there is at all times mixed, irrespective of infinitesimal fractions of unchanged anode, a preponderating quantity (about ten per cent. of the weight of the anode) of gold in an extremely fine state of division. The presence of this gold is due to the fact that a portion of the anode gold is at once converted into a protochlorid (AuCl) instead of being first converted into a chlorid, and the protochlorid is immediately after being formed broken up into a chlorid and finely-divided gold.

While, as described, a portion of the anode constituents pass over into the solution and another portion subsides in the form of an insoluble deposit, pure gold is exclusively deposited at the cathode, even from solutions of constantly-increasing impurity and with currents of a density of one thousand amperes per square meter. The gold extracted from the electrolyte at the cathode is therefore constantly replaced principally by gold dissolved at the anode and in part by equivalent quantities of other metals, and as the quantity of gold deposited at the cathode corresponds with the quantity of silver, lead, and bismuth converted into solid chlorids there is a gradual impoverishment of the electrolyte in gold, which is to be replaced by the addition of sufficient gold-chlorid solution.

65 The simultaneous accumulation of foreign constituents in the electrolyte does not affect the purity of the gold deposited, even if there

is an excess of such impurities, so long as the proper amount of gold is present in the electrolyte. In fact, the presence of these foreign constituents is even advantageous to the deposition of pure gold at the cathode in that although the deposit is very voluminous from pure solutions, especially when currents of high density are used, yet the compactness of the deposit without being in the least affected in its purity increases with the increase in the impurities in the electrolyte.

From what has been said it will be seen that the electrolytic extraction of gold can be continuously carried on with the least possible quantities of hydrochloric acid, while in the purification of gold by chemical means fresh acid is required for each batch of material treated, and not only this, but each solution must be treated with fresh quantities of precipitant. In my process the small quantity of hydrochloric acid necessary to the formation of the electrolyte in consequence of the separation of pure gold at the cathode is always available anew as a solvent. Hence this very small quantity of acid will cause or insure in a greater sequence of operations not only the dissolution of the gold, but also the precipitation from the solution of the pure gold contained therein. There is a further advantage in the continuous extraction of gold from like solutions in that it is possible to recover from large quantities of anode materials the comparatively small percentage of platinum contained therein in that after the precipitation of the gold the platinum may be directly recovered in the form of ammonio-chlorid. Thus, for instance, if the anode metal contains on an average one-thousandth part of platinum two kilos of this metal would be obtained in a hundred days from a daily working up of twenty kilos of anode metal. In view of the fact, as has been shown by practice, that the electrolyte may contain twice as much platinum as gold without affecting the purity of the cathode deposit it is obvious that the electrolyte can be used until the separation therefrom of its platinum constituent can be most advantageously effected. This, however, is not the case with palladium, although quantities of this metal equal to five grams per liter of the electrolyte will not appreciably affect the purity of the gold deposited at the cathode. The presence of a greater quantity will, however, affect the purity of said deposit in that traces of palladium become apparent therein. In view of the fact that the proportion of palladium in the anode metal is usually but a fraction of its platinum contents the electrolyte can be used as such until it contains platinum enough to warrant its advantageous separation.

In the carrying out of the invention it may be remarked in completion of what has been said that owing to the high value of the anode material and the solution, as well as of the product of the electrolysis, it is advantageous

that the work be performed within the shortest possible time and within the smallest possible space. Accordingly currents of the highest possible density and comparatively thin anodes should be made use of. Thus, for instance, if an anode four millimeters thick is used it will be so far consumed in twenty-four hours with an initial current density of four hundred amperes per square meter that the remainder, of about one-tenth the original weight, is preferably used in making fresh anodes.

The approximately uniform percentage of gold that goes over into the anode mud which collects on the bottom of the electrolytic apparatus is recovered therefrom either directly or after preliminary purification of the mud, according to its composition, and used as anode material. To this end the mud may be removed from the electrolytic apparatus either after each operation or after longer periods, as may be found necessary or advantageous.

The cathodes are made of thin rolled pure gold electrolytically obtained and may be of the same length as the anodes, but considerably narrower, because they rapidly increase in size in all directions under the action of the electric current, the deposit being a coherent one even with currents of a comparatively high initial density. This fact enables me, even with currents of high density, to place the electrodes in close proximity to each other, as within about three centimeters from each other, without danger of short-circuiting or danger of the cathode deposit being rendered impure.

At the beginning of the electrolytic operation, when the electrolyte is yet free or comparatively free from foreign matter or impurities and the deposition of gold at the cathode is comparatively voluminous, the electrodes must be arranged farther apart or the cathodes more frequently changed.

In the accompanying drawings I have illustrated an apparatus for practically carrying out my invention, showing the arrangement of the electrodes in their respective interconnected cells or vessels and combined with means for maintaining the level of the liquid in said cells or vessels, and in which—

Figure 1 is a vertical longitudinal sectional view of one of the vessels, and Fig. 2 a sectional plan view of a number of such connected in series.

Upon each vessel *v* for containing the electrolyte and electrodes is arranged a frame *w*, of wood, and upon the longer sides of said frame suitable conductive strips or bars *a* and *b*, of copper or brass, are secured, to which cross-bars, (numbered from 1 to 9, inclusive,) also of a conductive material, are alternately connected, and to said cross-bars the electrodes are electrically connected in such manner that the anode cross-bars 2 4 6 8 alternate with the cathode cross-bars 1, 3, 5, 7, and 9, connected with their respective conductive

strips *a* *b* by binding-posts *a'* *b'*. The anodes are indicated by the symbol A and the cathodes by the symbol C. The vessels *v* are connected in series through a conductive connection *c'* between the conductors *b* and *a* of two contiguous vessels, the conductors *a* and *b* of the first and last vessels of the series being respectively connected with the negative 75 and positive poles of a suitable source of electricity, as a dynamo.

The cells or vessels *v* are made of any suitable material capable of resisting the action of the electrolyte, and if the latter is heated 80 it is necessary, owing to loss by evaporation, to maintain it at a uniform level, to which end I arrange above the vessel *v* a reservoir *f*, containing an electrolyte such as is contained in said vessel, and from said reservoir 85 lead two pipes *m* and *n*, the reservoir being provided with a normally-closed filling-aperture. The pipe *m* has its outlet slightly below the surface of the electrolyte in vessel *v*, while the pipe *n* is a siphon-pipe that extends 90 near to the bottom of said reservoir *f* and supplies liquid to vessel *v* the moment the level sinks below the outlet of pipe *m* and allows air to enter the same, while the flow of liquid from the reservoir is stopped the moment the level of the electrolyte has risen to 95 seal the outlet of said pipe. The liquid used for compensating losses of the electrolyte by evaporation is preferably the water used in washing the gold deposits and the residues 100 and mud taken from the cells, of which water there is generally a sufficient quantity available; but should this not be the case the deficiency is made up with distilled water. In this manner I am enabled to return to the 105 electrolyte the diluted portion of the gold solution taken therefrom without previously concentrating the same, as this is effected by the evaporation of the hot electrolyte during the electrolytic operation.

In the extraction of chemically pure gold from alloys of such it must be borne in mind that in the chlorination of the anode constituents other than gold an equivalent quantity of the latter metal is separated from the 115 electrolyte at the cathode, which must be replaced by addition of gold chlorid. With such materials it will be necessary to supplement the electrolytical process by chemical processes in proportion as the quantity of the 120 components of the gold alloy other than gold is greater or less and as the electrochemical equivalent thereof relatively to gold is lower. If the anode material contains a comparatively great quantity of silver, the anode-surface will be coated therewith in the form of a non-conductive chlorid that does not readily drop off, thereby reducing the active area of the anode, giving rise to the evolution of gaseous chlorin, so that the anode will be 125 insufficiently attacked and the gold in solution will be precipitated. In electrolyzing alloys of this kind the interruption of the operation by the deposition of chlorid of silver

at the anode can readily be avoided by removal of said chlorid mechanically, as by means of a spatula, which operation is performed periodically, the frequency depending upon the percentage of silver in the alloy and the density of the electric current. This also applies in case bismuth is present in the alloy, and if the latter also contains a considerable amount of lead the acid solution becoming rapidly saturated with lead chlorid, and as soon as this is the case both electrodes, as well as the internal surfaces of the cell or vessel and the surface of the solution or electrolyte, become coated with lead-chlorid crystals. Although in this case it is possible to obtain the precipitated gold free from lead by repeated boiling in distilled water and that the greater portion of the lead chlorid may be removed from the cold electrolyte by scooping it out, yet an electrolyte thus charged with impurities is not adapted for continuous operation. This can also be avoided by adding to the electrolyte a sufficiency of sulfuric acid to convert the lead chlorid into sulfate, and to this end I add to the electrolyte a quantity of concentrated sulfuric acid equal to the quantity of free hydrochloric acid present. The lead then forms on the anode an almost insoluble deposit of lead sulfate, which gradually drops off or which, as in the case of silver, is mechanically removed when lead is present at the anode in considerable quantities.

Of course it will be understood that the sulfuric acid consumed in the formation of the lead sulfate will have to be replaced from time to time and that whenever the anode material is supposed to contain lead it is advisable to add sulfuric acid to the electrolyte, especially as this acid does not exert a deleterious influence on the electrolytic actions.

Having thus described my invention, what I claim as new therein, and desire to secure by Letters Patent, is—

1. The herein-described process, which consists in passing an electric current from an anode of impure gold or of an auriferous alloy through a gold-chlorid solution, to a suitable cathode, and maintaining in said solution at all times during the passage of such current hydrochloric acid in sufficient quantity to prevent the liberation of gaseous chlorin at the anode, for the purpose set forth.

2. The herein-described process, which consists in passing an electric current from an

anode of impure gold or of an auriferous alloy through a heated gold-chlorid solution to a suitable cathode, and maintaining in said solution at all times during the passage of such current hydrochloric acid in sufficient quantity to prevent the liberation of gaseous chlorin at the anode, for the purpose set forth. 60

3. The herein-described process, which consists in passing a current of high density (five hundred amperes per square meter or higher) 65 from an anode of impure gold or of an auriferous alloy through a gold-chlorid solution to a suitable cathode, and maintaining in said solution at all times during the passage of such current hydrochloric acid in sufficient quantity to prevent the liberation of gaseous chlorin at the anode, for the purpose set forth. 70

4. The herein-described process, which consists in passing a current of high density (five hundred amperes per square meter or higher) 75 from an anode of impure gold or of an auriferous alloy through a heated gold-chlorid solution to a suitable cathode, and maintaining in said solution at all times during the passage of such current hydrochloric acid in sufficient quantity to prevent the liberation of gaseous chlorin at the anode, for the purpose set forth. 80

5. The herein-described process which consists in passing an electric current from an anode of impure gold or of an auriferous alloy to a suitable cathode through a gold-chlorid solution and maintaining in said solution sulfuric acid, together with hydrochloric acid in sufficient quantity to prevent the liberation of gaseous chlorin at the anode during 90 the electrolytic action, for the purpose set forth. 85

6. The herein-described process, which consists in passing an electric current from an anode of impure gold or of an auriferous alloy through a heated gold-chlorid solution to a suitable cathode, and maintaining in said solution sulfuric acid, together with hydrochloric acid in sufficient quantity to prevent the liberation of gaseous chlorin at the anode during 100 the electrolytic action, for the purpose set forth.

In testimony that I claim the foregoing as my invention I have signed my name in presence of two subscribing witnesses.

EMIL WOHLWILL.

Witnesses:

MARCO SALOMON,  
ADOLPH BENON.